

J. A. DUBBS.

TREATING PETROLEUM AND PETROLEUM RESIDUES.

APPLICATION FILED DEC. 5, 1910.

1,057,227.

Patented Mar. 25, 1913.



WITNESSES:

Theodore Duff  
J. Herbert Bradley.

INVENTOR

Jesse A. Dubbs  
by Christy and Christy

# UNITED STATES PATENT OFFICE.

JESSE A. DUBBS, OF LOS ANGELES, CALIFORNIA.

## TREATING PETROLEUM AND PETROLEUM RESIDUES.

1,057,227.

Specification of Letters Patent.

Patented Mar. 25, 1913.

Application filed December 5, 1910. Serial No. 595,750.

*To all whom it may concern:*

Be it known that I, JESSE A. DUBBS, residing at Los Angeles, in the county of Los Angeles and State of California, a citizen 5 of the United States, have invented or discovered certain new and useful Improvements in Treating Petroleum and Petroleum Residues, of which improvements the following is a specification.

10 My invention relates to improvements in the treatment of petroleum and petroleum residues to produce an asphalt for commercial purposes. By "petroleum residues" I mean to indicate those substances which remain in the still chamber after the lighter gases and oils have been removed from the petroleum by distillation. The production of asphalt by the distillation of petroleum and of petroleum residues by distillation is 15 well known and needs no description. In the course of the operation of distillation to this end it has been customary for one purpose or another to blow through the liquid material in the still a blast of air, and for 20 some purposes also the liquid has been blown through with a blast of steam. I have found that these in-blown fluids have each of them its peculiar effect upon the asphalt produced. If the material, while being distilled, is 25 blown with steam, the resulting asphalt will be one of relatively great plasticity and ductility. If, on the other hand, the material is blown with air during distillation, the resulting asphalt will be hard and brittle 30 and lacking in ductility.

35 I have found it advantageous (and my present invention consists in such operation) to blow the material while under treatment, throughout a substantial portion of the operation of distillation simultaneously with both fluids. The asphaltum which I produce by such operation is neither too plastic, as is the case with steam-blown asphalt, nor is it too brittle, as is the case with air-blown asphalt.

40 My invention further resides in so controlling the supply of steam and air employed for this purpose, and so relating the quantities of injected fluids the one to the other, that the product is within my control, so far as concerns ductility and plasticity; and I may vary the degree of ductility of the product to better adapt the product for specific uses. Furthermore, in

dealing with petroleums and petroleum residues of different grades and characters, by varying the relative and absolute quantities of the in-blown fluids, I am able to produce a product coming up to certain requirements.

45 I shall describe first a typical operation upon a fairly representative article, and as a sequel describe how the operation may be varied.

50 I take, for example, California crude petroleum, having a specific gravity of 18° Baumé at atmospheric temperature. I place this petroleum in a still of any preferred construction having proper pipe connections, and bring it to a temperature of 70 225° F. by the application of external heat. I then begin to inject steam, preferably through a perforated pipe at the bottom of the still, in a well known manner, to obtain distribution of the injected steam throughout the body of the charge in the still. The 55 initial temperature of the steam may be approximately 225° F. At first the steam is introduced in limited quantities, to avoid boiling over of the contents; but once the 60 still gets to running regularly and smoothly, the volume of introduced steam is increased, until the volume of distillate produced is in suitable relation to the quantity of material under treatment. After a period, which will 65 ordinarily cover two or three hours, air also is introduced. The air may be blown in either through a separate perforated pipe or through the same pipe which carries the 70 steam; but, if the air and steam are mingled, 75 it is preferable that the air be preheated before it is introduced into the flow of steam, as otherwise it will effect some condensation of the steam. To prevent such condensation, the temperature of the in-blown air will be 80 approximately that of the steam. The air also is introduced in a gradually increasing 85 volume until, as compared with the amount of steam, the volume of air introduced will 90 be from 50% to 75% of the other fluid, and 95 the relative amount will be determined by observation in view of the results to be reached. The temperature at the time the air is introduced under such circumstances will be between 250° and 300° F. ordinarily. 100 From this point on, the operation continues 105 with the combined air and steam blasts until distillation is finished. This will be

after an interval of about twenty four to thirty six hours (depending upon the degree of hardness to which the asphalt is to be brought), and the ultimate temperature will 5 be between 400° and 650° F. (this also depending upon the quality of the product desired).

When the distillation is substantially finished, the air is first shut off and the steam 10 is allowed to continue to pass through the oil for about half an hour, or until such time as vapors which might otherwise condense in the still chamber are carried out of the still. The primary object of this prolonged action 15 of the steam is to render the product practically odorless.

The accompanying drawing will illustrate 20 my invention, this being a view in vertical section of a still for carrying the invention into practice.

The still itself is indicated at 1; a suitable furnace or burner is indicated at 2. It will be understood that, while, (as hereinbefore described) the burner 2 will afford the initial 25 heat, continuation of heat may be had by the internal combustion following upon the introduction of air when the material is still at elevated temperature. Whether the heat of the burner 2 be continued throughout the 30 operation is a detail which is variable within the judgment of the operator, for it is a matter within the common knowledge of the art at the present day. The pipe for the introduction of steam and air is indicated at 35 3, and is forked as at 6 in order to have connection to steam and air supply pipes. Within the still chamber the pipe 3 terminates in a perforated distributing-head 4. The distillates from the chamber 1 escape 40 from the top thereof by means of the passageway 5.

My understanding of the matter is this. The asphalt is to be considered to be made up of two elements, one commonly called 45 asphaltene and the other petroleum. Asphaltene is the hard element of the mixture and petroleum the fluid element. In other words, asphaltene is a solid held in solution in the more or less fluid petroleum. When 50 petroleum is blown with steam the petroleum element predominates in the product, and when it is blown with air the asphaltene element predominates.

If the material which is treated is one that 55 does not under normal treatment afford an asphalt of sufficient hardness, then the blowing in of air may be begun at or shortly after, or if need be even before the blowing in of the steam begins, and the volume of 60 the air relative to the volume of steam to be introduced may be increased. If, on the other hand, the character of the substance treated is such that asphalt produced therefrom under normal conditions is too hard, 65 then the time for introducing the air may be

delayed or the quantity of air to be introduced may be diminished, or both, to afford a softer product.

So long as steam is present in an amount as great as 25% of the air, an explosive mixture cannot be formed in the still chamber. If however the relative amount of steam falls below that minimum, precautions should be taken in the manner known to the art to prevent explosion. 70

The operation described above is based 75 upon the assumption that the oil is initially free from water. If however the oil to be treated does contain water, it should first be dried in any preferred manner, before my 80 operation herein described is performed upon it.

I have referred above to petroleum and 85 petroleum residue. It will be understood that petroleum residue is a result of an initial distillation of petroleum itself, and no separate explanation is necessary to enable one skilled in the art to treat either or both substances. Consequently, residual products such as petroleum tar and other products 90 from which the lighter distillates, or the greater percentage of the original petroleum has been taken are susceptible to this process in the same manner and the same degree as are those petroleum substances which have 95 still a large proportion of readily distillable ingredients present in them. Where the residual products consist of petroleum tar and like heavy residues, these residues are preferably first subjected to heat until 100 brought to a temperature of 300° to 450° F., before the blasts are introduced.

I claim herein as my invention:

1. The method herein described of producing asphalt from petroleum and petroleum residues, which consists in distilling away the lighter ingredients of the substance under treatment and as such distillation progresses blowing the mass under treatment simultaneously with blasts of 110 steam and of air.

2. The method herein described of producing asphalt from petroleum or petroleum residue, which consists in distilling away the lighter components of the substance to 115 be treated, and during such operation of distillation blowing the substance under treatment with blasts of air and of steam in relatively regulated quantities according to the physical properties desired in the product. 120

3. The method of treating petroleum and residual petroleum products to obtain asphalt and asphaltic products which consists in injecting in the heated body under treatment, steam and air in mingled condition in 125 proportions and quantities regulable according to the product desired.

4. The method of treating petroleum tar or residual petroleum products to obtain asphalt and asphaltic products, which consists 130

in heating the residue from 300 to 450 degrees F., then blowing the petroleum residue with air and later introducing steam, varying the proportions of the steam and air for 5 producing softer or harder products.

5. The method of treating petroleum and residual petroleum products, which consists in blowing the heated petroleum or its products with steam and then introducing air 10 conjointly with the steam, to obtain harder or softer products, the quantity of steam with the air for softer products being inversely proportional to the quantity of air with the steam for harder products.

15 6. The method herein described of preparing asphalt from petroleum or petroleum residue, which consists in distilling away

the lighter ingredients of the material acted upon, and in the course of such distillation introducing into the material successively 20 blasts of steam and of air, and continuing the operation with the conjoint blowing in of both fluids, the order in which the blasts are successively introduced and the interval of time between their successive introduction 25 being determined according to the physical properties desired in the product.

In testimony whereof, I have hereunto set my hand.

JESSE A. DUBBS.

Witnesses:

ANTON GLOETZNER, Jr.,  
F. J. McCCLARY.